

## UNITED STATES PATENT OFFICE

2,236,852

PROCESS FOR PRODUCING ENAMEL,  
MORE PARTICULARLY WHITE CLOUDED  
ENAMEL

Ignaz Kreidl, Cleveland, Ohio

No Drawing. Application August 3, 1937, Serial  
No. 157,229. In Austria March 4, 1937

6 Claims. (Cl. 106—36.2)

In the production of enamel, such as for example iron enamel, more particularly white clouded iron enamel, the properties of the slip play an important role in wet enameling. In the production of the slip the enamel frit is ground with addition of water. During the grinding, in order to obtain a satisfactory applying capability for the product, usually clay is added, and in fact for coating or covering enamels usually in a quantity of 6-10%. The grinding usually takes place with a quantity of water which is as small as possible in order to render it possible to give the mass the desired consistency for the application by dilution. If an enamel is made up with too much water then the resulting slip is too thin and the enamel "runs" as one says in the art, or it "stays" only very badly. However such "running" of the enamel frequently occurs even without excessive water addition. Such "running" enamels are very bad to apply.

In order now to bring such enamel to a condition or to bring it again to a condition so that it will "stay," one has recourse to so-called adjusting agents. The adjusting action of these agents exerts itself in a thickening of the enamel slip, which is of varying degree with the different adjusting agents, but in certain substances may go so far that the slip sets to a stiff mass which can be no longer worked by the wet enameling process. As such adjusting agents exclusively electrolytes come into consideration, e. g. chlorides and sulphates of magnesium and ammonium, carbonates, and so forth.

However by varying the composition of the enamel frit one can also arrive at slips which stay too strongly and therefore cannot be satisfactorily worked by the wet enameling process or at least are no longer compatible with, or are not influenced by, additions having an adjusting action. This is more particularly important inasmuch as for covering or coating enamel in addition to clay the clouding agent is also added on the mill and many clouding agents or other indispensable additions exert an adjusting action on the mill—i. e. set up the slip—and by this action impair the applicability of the enamel slip. More particularly this plays a role in gas cloudings for which also clouding agents come into consideration which are capable of exerting an adjusting effect, so that for such gas clouding agents on the one hand enamel frits which in the slip already "stay" strongly cannot be satisfactorily worked up, on the other hand, slips also are disadvantageous which already with indispensable additions

are too strong "staying" and therefore cannot be satisfactorily worked up.

Such slips which "stay" too strongly and which cannot be worked up forthwith in the wet process, more particularly slips in which this too strong staying power is caused either by the composition of the enamel frit or by indispensable additions on the mill, or both by such additions as well as by the composition of the frit, also cannot be made capable of application by dilution with water. Even if one can obtain sufficient viscosity by addition of water then in the case of such slips, a coating free from streaks is not possible. It is, however, possible to obtain a coating free from streaks by diluting correspondingly more strongly, but such strong dilution has the effect that only insufficient layer thicknesses can be obtained, that is to say the layer thickness is too small. Moreover drawbacks arise during drying when using such slips.

The present invention depends upon the discovery that in the case of such slips having too powerful staying power, more particularly such slips of too strong staying power which by dilution alone cannot be brought to the necessary state of adjustment, the cause for this phenomenon obviously lies in the too high thixotropy.

According to the invention these drawbacks brought about by too high thixotropy of the slip are removed by the addition of certain electrolytes having action contrary to that of the adjusting effect. The invention in fact depends upon the discovery that by addition of certain substances to the slip an action can be attained contrary to the adjusting effect, whereby the invention affords a means of adjusting down slips of too high staying power without excessively increasing the water addition, and in fact even with small water addition.

This action according to the invention is produced by the use of polyvalent (polybasic) strong acids and in fact the better the higher their basicity for the same activity, and in fact more particularly the tribasic inorganic and the di- and poly-basic organic acids and mixtures of such.

According to the invention also, such acid salts may be employed which correspond to the above-mentioned conditions.

Oxalic acid on the one hand, phosphoric acid on the other hand, or mixtures of these substances, best conform to the requirements.

The quantities to be used are found empirically and lie between about 1 and 5%.

This invention accordingly enables the field of practical applicability for enamel slips to be

considerably widened. On the one hand such slips may be made utilisable for the enameling which in consequence of too powerful staying power hitherto could not be worked or only with difficulty, and on the other hand the slips capable of being worked up in the usual manner can be improved in their applicability and the working up of the same with additions on the mill can be made possible, which hitherto were out of the question owing to the adjusting action attending the same. Thus the invention favours the use of enamel frits which in consequence of their composition yield enamel slips of powerful staying powers, such as more particularly enamel frits, which in the slip show an enhanced colloidal character as compared with normal enamel frits, such as for example enamel frits, which show a fluorine content of about 10% and more fluorine originating from fluorine compounds which do not contain aluminium. The invention also enables electrolytes or substances to be used in spite of their undesired adjusting action.

In the process according to the present invention, finally there is the advantage that a uniform drying of the slip applied is ensured.

The process according to the invention is more particularly suitable for the production of gas clouded enamel by means of enamel slips which contain enamel frits which as compared with normal frits show in the slip an enhanced colloidal character.

cially slips for white clouded iron enamel tending to become excessively stiff, comprising reducing the setting of said slips by the addition of phosphoric acid, in a quantity ranging approximately between 1 to 5 parts per thousand.

2. A process for preparing enamel slips, especially slips for white clouded iron enamel tending to become excessively stiff, comprising reducing the setting of said slips by the addition 10 of oxalic acid, in a quantity ranging approximately between 1 to 5 parts per thousand.

3. In a process of preparing enamel slips comprising adding to said slips at least one substance capable of reducing the stiffness of said slips and selected from the group consisting of polybasic acids and acid reacting salts thereof, in a quantity ranging between 1 to 5 parts per thousand of the said slips.

4. An enamel slip of controlled stiffness having incorporated therewith phosphoric acid in a quantity between about 1 to 5 parts per thousand parts of said slip.

5. An enamel slip of controlled stiffness having incorporated therewith oxalic acid in a quantity between about 1 to 5 parts per thousand parts of said slip.

6. An enamel slip of controlled stiffness having incorporated therewith at least one substance capable of reducing the stiffness of said slip and selected from the group consisting of polybasic acids and acid reacting salts thereof in a quantity ranging between 1 to 5 parts per thousand of the said slip.

IGNAZ KREIDL.